# EUROPEAN PATENT SPECIFICATION

(11) **EP 2 997 172 B1**
(45) Date of publication and mention of the grant of the patent: **26.08.2020**
(21) Application number: 14729827.7
(22) Date of filing: 16.05.2014
(51) Int. Cl.: C22C 38/02, C22C 38/38, C22C 38/34, C22C 38/32, C22C 38/06, C21D 9/46, C23C 2/06, C23C 2/02, C21D 8/02, C22C 38/18, C22C 38/00, C22C 38/12, C22C 38/04, C21D 1/78, C21D 6/00, C23C 2/40, C21D 1/18

(54) **METHOD OF PRODUCTON OF A HIGH STRENGTH STEEL EXHIBITING GOOD DUCTILITY VIA QUENCHING AND PARTITIONING TREATMENT BY ZINC BATH**
HERSTELLUNG EINES HOCHFESTEN STAHLS MIT GUTER DUKTILITÄT MITTELS ABSCHRECK- UND PARTITIONIERUNGSBEHANDLUNG DURCH EIN ZINKBAD
PROCÉDÉ DE PRODUCTION D'UN ACIER À HAUTE RÉSISTANCE MÉCANIQUE ET À BONNE DUCTILITÉ PAR TRAITEMENT DE TREMPE ET DE PARTITIONNEMENT EN BAIN DE ZINC

(30) Priority: 17.05.2013 US 201361824699 P; 17.05.2013 US 201361824643 P
(43) Date of publication of application: 23.03.2016
(73) Proprietor: Ak Steel Properties, Inc., West Chester, OH 45069 (US)
(72) Inventor: THOMAS, Grant, Aaron, Liberty Township, OH 45011 (US); GARZA-MARTINEZ, Luis, G., Wyoming, OH 45215 (US)
(74) Representative: Samson & Partner Patentanwälte mbB
(86) International application number: PCT/US2014/038425
(87) International publication number: WO 2014/186722

(56) References cited:
- EP-A1- 2 258 886
- EP-A1- 2 325 346
- EP-A1- 2 325 346
- EP-A1- 2 524 970
- EP-A1- 2 524 970
- WO-A1-2004/022794
- WO-A1-2011/111332
- WO-A1-2012/120020

## Description

The present application claims priority from provisional patent application serial no. 61/824,643, entitled "High-Strength Steel Exhibiting Good Ductility and Method of Production via In-Line Partitioning Treatment by Zinc Bath," filed on May 17, 2013; and provisional patent application serial no. 61/824,699, entitled "High-Strength Steel Exhibiting Good Ductility and Method of Production via In- Line Partitioning Treatment Downstream of Molten zinc Bath," filed on May 17, 2013.

### BACKGROUND

It is desirable to produce steels with high strength and good formability characteristics. However, commercial production of steels exhibiting such characteristics has been difficult due to factors such as the desirability of relatively low alloying additions and limitations on thermal processing capabilities of industrial production lines. The present invention relates to steel compositions and processing methods for production of steel using hot-dip galvanizing/galvannealing (HDG) processes such that the resulting steel exhibits high strength and cold formability.

EP 2325 346 A1 relates to a high-strength steel sheet used in industrial fields such as automobiles and electrics and having ductility and stretch-flangeability, and a tensile strength (TS) of 980 MPa or more.

EP 2 524 970 A1 discloses a steel sheet with a production method for a steel sheet, which method comprises a hotdip galvanizing/galvannealing step.

### SUMMARY

The invention relates in one aspect to a method for producing a hot dip galvanized/galvannealed steel sheet, the steel sheet consisting of the following elements by weight percent: 0.15-0.5% carbon; 1-3% manganese;
2% or less silicon, aluminum, or some combination thereof; 0.5% or less molybdenum; 0.05% or less niobium; and the balance being iron and other incidental impurities; or
0.15-0.4% carbon; 1.5-4% manganese; 2% or less silicon, aluminum, or some combination thereof;
0.5% or less molybdenum; 0.05% or less niobium; and the balance being iron and other incidental impurities;
wherein the method comprising the steps of:
(a) heating the steel sheet to a first temperature (T1), wherein T1 is at least above the temperature at which the steel sheet transforms to austenite and ferrite;
(b) cooling the steel sheet to a second temperature (T2) by cooling at a cooling rate, wherein T2 is below the martensite start temperature (Mₛ), wherein the cooling rate is sufficiently rapid to transform austenite to martensite, to avoid the formation of non-martensitic transformation products;
(c) re-heating the steel sheet to a partitioning temperature, wherein the partitioning temperature is sufficient to permit diffusion of carbon within the structure of the steel sheet;
(d) stabilizing austenite by holding the steel sheet at the partitioning temperature for a holding time, wherein the holding time is of a period of time sufficient to permit diffusion of carbon from martensite to austenite;
(e) subjecting the steel sheet to a hot dip galvanizing or galvannealing process during the step of stabilizing austenite; and
(f) cooling the steel sheet to room temperature.

The present steel is produced using the above indicated composition and modified HDG process that together produces a resulting microstructure consisting of generally martensite and austenite (among other components, wherein the formation of non-martensitic transformation products is avoided). To achieve such a microstructure, the composition includes certain alloying additions and the HDG process includes certain process modification, all of which are at least partially related to driving the transformation of austenite to martensite followed by a partial stabilization of austenite at room-temperature.

### BRIEF DESCRIPTION OF THE FIGURES

The accompanying figures, which are incorporated in and constitute a part of this specification, illustrate embodiments, and together with the general description given above, and the detailed description of the embodiments given below, serve to explain the principles of the present disclosure.
FIGURE 1 depicts a schematic view of a HDG temperature profile with a partitioning step performed after galvanizing/galvannealing. This HDG temperature profile is not part of the present invention.
FIGURE 2 depicts a schematic view of a HDG temperature profile with a partitioning step performed during galvanizing/galvannealing.
FIGURE 3 depicts a plot of one embodiment with Rockwell hardness plotted against cooling rate.
FIGURE 4 depicts a plot of another embodiment with Rockwell hardness plotted against cooling rate.
FIGURE 5 depicts a plot of another embodiment with Rockwell hardness plotted against cooling rate.
FIGURE 6 depicts six photo micrographs of the embodiment of FIG. 3 taken from samples being cooled at various cooling rates.
FIGURE 7 depicts six photo micrographs of the embodiment of FIG. 4 taken from samples being cooled at various cooling rates.
FIGURE 8 depicts six photo micrographs of the embodiment of FIG. 5 taken from samples being cooled at various cooling rates.
FIGURE 9 depicts a plot of tensile data as a function of austenitization temperature for several embodiments.
FIGURE 10 depicts a plot of tensile data as a function of austenitization temperature for several embodiments.
FIGURE 11 depicts a plot of tensile data as a function of quench temperature for several embodiments.
FIGURE 12 depicts a plot of tensile data as a function of quench temperature for several embodiments.

### DETAILED DESCRIPTION

FIG. 1 shows a schematic representation of the thermal cycle used to achieve high strength and cold formability in a steel sheet having a certain chemical composition (described in greater detail below) as a comparative example. In particular, FIG. 1 shows a typical hot-dip galvanizing or galvannealing thermal profile (10) with process modifications shown with dashed lines. In one embodiment the process generally involves austenitization followed by a rapid cooling to a specified quench temperature to partially transform austenite to martensite, and the holding at an elevated temperature, a partitioning temperature, to allow carbon to diffuse out of martensite and into the remaining austenite, thus, stabilizing the austenite at room temperature. In some embodiments, the thermal profile shown in FIG. 1 may be used with conventional continuous hot-dip galvanizing or galvannealing production lines, although such a production line is not required.

As can be seen in the comparative example of FIG. 1, the steel sheet is first heated to a peak metal temperature (12). The peak metal temperature (12) in the illustrated example is shown as being at least above the austenite transformation temperature (A₁) (e.g., the dual phase, austenite + ferrite region). Thus, at the peak metal temperature (12), at least a portion of the steel will be transformed to austenite. Although FIG. 1 shows the peak metal temperature (12) as being solely above A₁, it should be understood that in some embodiments the peak metal temperature may also include temperatures above the temperature at which ferrite completely transforms to austenite (A₃) (e.g., the single phase, austenite region).

Next the steel sheet undergoes rapid cooling in the comparative example. As the steel sheet is cooling, some embodiments may include a brief interruption in cooling for galvanizing or galvannealing. In embodiments where galvanizing is used, the steel sheet may briefly maintain a constant temperature (14) due to the heat from the molten zinc galvanizing bath. Yet in other embodiments, a galvannealing process may be used and the temperature of the steel sheet may be slightly raised to a galvannealing temperature (16) where the galvannealing process may be performed. Although, in other comparative examples, the galvanizing or galvannealing process may be omitted entirely and the steel sheet may be continuously cooled.

The rapid cooling of the steel sheet in the comparative example is shown to continue below the martensite start temperature (Mₛ) for the steel sheet to a predetermined quench temperature (18). It should be understood that the cooling rate to Mₛ may be high enough to transform at least some of the austenite formed at the peak metal temperature (12) to martensite. In other words the cooling rate may be rapid enough to transform austenite to martensite instead of other non-martensitic constituents such as ferrite, pearlite, or bainite which transform at relatively lower cooling rates.

As is shown in the comparative example of FIG. 1, the quench temperature (18) is below Ms. The difference between the quench temperature (18) and Mₛ may vary depending on the individual composition of the steel sheet being used. However, in many embodiments the difference between quench temperature (18) and Mₛ may be sufficiently great to form an adequate amount of martensite to act as a carbon source to stabilize the austenite and avoid creating excessive "fresh" martensite upon final cooling. Additionally, quench temperature (18) may be sufficiently high to avoid consuming too much austenite during the initial quench (e.g., to avoid excessive carbon enrichment of austenite greater than that required to stabilize austenite for the given embodiment).

In many embodiments, quench temperature (18) may vary from about 191 °C to about 281 °C, although no such limitation is required. Additionally, quench temperature (18) may be calculated for a given steel composition. For such a calculation, quench temperature (18) corresponds to the retained austenite having an Mₛ temperature of room temperature after partitioning. Methods for calculating quench temperature (18) are known in the art and described in J. G. Speer, A. M. Streicher, D. K. Matlock, F. Rizzo, and G. Krauss, "Quenching And Partitioning : A Fundamentally New Process to Create High Strength Trip Sheet Microstructures," Austenite Formation and Decomposition, pp. 505-522, 2003; and A. M. Streicher, J. G. J. Speer, D. K. Matlock, and B. C. De Cooman, "Quenching and Partitioning Response of a Si-Added TRIP Sheet Steel," in Proceedings of the International Conference on Advanced High Strength Sheet Steels for Automotive Applications, 2004.

The quench temperature (18) may be sufficiently low (with respect to Mₛ) to form an adequate amount of martensite to act as a carbon source to stabilize the austenite and avoid creating excessive "fresh" martensite upon the final quench. Alternatively, the quench temperature (18) may be sufficiently high to avoid consuming too much austenite during the initial quench and creating a situation where the potential carbon enrichment of the retained austenite is greater than that required for austenite stabilization at room temperature. In some embodiments, a suitable quench temperature (18) may correspond to the retained austenite having an Mₛ temperature of room temperature after partitioning. Speer and Streicher *et al.* (above) have provided calculations that provide guidelines to explore processing options that may result in desirable microstructures. Such calculations assume idealized full partitioning, and may be performed by applying the Koistinen-Marburger (KM) relationship twice (*fₘ* = 1-*e*^{-1.1*x*10⁻²(Δ*T*)}) - first to the initial quench to quench temperature (18) and then to the final quench at room temperature (as further described below). The Ms temperature in the KM expression can be estimated using empirical formulae based on austenite chemistry (such as that of Andrew's linear expression):

*Ms*(°*C*) = 539 - 423C - 30.4*Mn* - 7.5*Si* + 30*Al*

The result of the calculations described by Speer et al. may indicate a quench temperature (18) which may lead to a maximum amount of retained austenite. For quench temperatures (18) above the temperature having a maximum amount of retained austenite, significant fractions of austenite are present after the initial quench; however, there is not enough martensite to act as a carbon source to stabilize this austenite. Therefore, for the higher quench temperatures, increasing amounts of fresh martensite form during the final quench. For quench temperatures below the temperature having a maximum amount of retained austenite, an unsatisfactory amount of austenite may be consumed during the initial quench and there may be an excess amount of carbon that may partition from the martensite.

Once the quench temperature (18) is reached, the temperature of the steel sheet is either increased relative to the quench temperature or maintained at the quench temperature for a given period of time. In particular, this stage is referred to as the partitioning stage. In such a stage, the temperature of the steel sheet is at least maintained at the quench temperature to permit carbon diffusion from martensite formed during the rapid cooling and into any remaining austenite. Such diffusion may permit the remaining austenite to be stable (or meta-stable) at room temperature, thus improving the mechanical properties of the steel sheet.

According to a further disclosure, the steel sheet may be heated above Mₛ to a relatively high partitioning temperature (20) and thereafter held at the high partitioning temperature (20). A variety of methods may be utilized to heat the steel sheet during this stage. By way of example only, the steel sheet may be heated using induction heating, torch heating, and/or the like. Alternatively, in other embodiments, the steel sheet may be heated but to a different, lower partitioning temperature (22) which is slightly below Mₛ. The steel sheet may then be likewise held at the lower partitioning temperate (22) for a certain period of time. In still a third alternative embodiment, another alternative partitioning temperature (24) may be used where the steel sheet is merely maintained at the quench temperature. Of course, any other suitable partitioning temperature may be used as will be apparent to those of ordinary skill in the art in view of the teachings herein.

After the steel sheet has reached the desired partitioning temperature (20, 22, 24), the steel sheet is maintained at the desired partitioning temperature (20, 22, 24) for a sufficient time to permit partitioning of carbon from martensite to austenite in the additional process disclosed herein. The steel sheet may then be cooled to room temperature.

FIG. 2 shows an alternative embodiment of the thermal cycle described above with respect to FIG. 1 (with a typical galvanizing/galvannealing thermal cycle shown with a solid line (40) and departures from typical shown with a dashed line). In particular, in this embodiment of the invention, like with the process of FIG. 1, the steel sheet is first heated to a peak metal temperature (42). The peak metal temperature (42) in the illustrated embodiment is shown as being at least above A₁. Thus, at the peak metal temperature (42), at least a portion of the steel sheet will be transformed to austenite. Of course, like the process of FIG. 1, the present embodiment may also include a peak metal temperature in excess of A₃.

Next, the steel sheet is rapidly quenched (44). It should be understood that the quench (44) needs to be rapid enough to initiate transformation of some of the austenite formed at the peak metal temperature (42) into martensite, thus avoiding excessive transformation to non-martensitic constituents such as ferrite, pearlite, banite, and/or the like.

The quench (44) is then ceased at a quench temperature (46). Like the process of FIG. 1, quench temperature (46) is below Mₛ. Of course, the amount below Ms may vary depending upon the material used. However, as described above, in the present invention the difference between quench temperature (46) and Mₛ needs to be sufficiently great to form an adequate amount of martensite yet be sufficiently low to avoid consuming too much austenite.

The steel sheet is then subsequently reheated (48) to a partitioning temperature (50, 52). Unlike the process of FIG. 1, the partitioning temperature (50, 52) in the present embodiment may be characterized by the galvanizing or galvannealing zinc bath temperature (if galvanizing or galvannealing is so used). For instance, in embodiments where galvanizing is used, the steel sheet may be re-heated to the galvanizing bath temperature (50) and subsequently held there for the duration of the galvanizing process. During the galvanizing process, partitioning may occur similar to the partitioning described above. Thus, the galvanizing bath temperature (50) may also function as the partitioning temperature (50). Likewise, in embodiments where galvannealing is used, the process may be substantially the same with the exception of a higher bath/partitioning temperature (52).

Finally, the steel sheet is permitted to cool (54) to room temperature where at least some austenite may be stable (or meta-stable) from the partitioning step described above.

In some embodiments the steel sheet may include certain alloying additions to improve the propensity of the steel sheet to form a primarily austenitic and martensitic microstructure and/or to improve the mechanical properties of the steel sheet. According to the invention, the steel sheets comprise the following, by weight percent: 0.15-0.4% carbon, 1.5-4% manganese, 0-2% silicon or aluminum or some combination thereof, 0-0.5% molybdenum, 0-0.05% niobium, other incidental elements, and the balance being iron.

Alternatively the compositions of the steel sheet includes of the following, by weight percent: 0.15-0.5% carbon, 1-3% manganese, 0-2% silicon or aluminum or some combination thereof, 0-0.5% molybdenum, 0-0.05% niobium, other incidental elements, and the balance being iron. Additionally, other embodiments falling outside the claimed steel compositions may include additions of vanadium and/or titanium in addition to, or in lieu of niobium, although such additions are entirely optional.

According to the invention carbon is used to stabilize austenite. For instance, increasing carbon may lower the Ms temperature, lower transformation temperatures for other non-martensitic constituents (e.g., bainite, ferrite, pearlite), and increase the time required for non-martensitic products to form. Additionally, carbon additions may improve the hardenability of the material thus retaining formation of non-martensitic constituents near the core of the material where cooling rates may be locally depressed. However, it should be understood that carbon additions may be limited as significant carbon additions may lead to detrimental effects on weldability.

According to the invention manganese provides additional stabilization of austenite by lowering transformation temperatures of other non-martensitic constituents, as described above. Manganese may further improve the propensity of the steel sheet to form a primarily austenitic and martensitic microstructure by increasing hardenability.

In other embodiments molybdenum may be used to increase hardenability.

In other embodiments silicon and/or aluminum may be provided to reduce the formation of carbides. It should be understood that a reduction in carbide formation may be desirable in some embodiments because the presence of carbides may decrease the levels of carbon available for diffusion into austenite. Thus, silicon and/or aluminum additions may be used to further stabilize austenite at room temperature.

In general, nickel, copper, and chromium may be used to stabilize austenite. For instance, such elements may lead to a reduction in the Mₛ temperature. Additionally, nickel, copper, and chromium may further increase the hardenability of the steel sheet.

In general niobium or titanium may be used to increase the mechanical properties of the steel sheet. For instance, niobium may increase the strength of the steel sheet through grain boundary pinning resulting from carbide formation.

Generally, in the production of steel sheets, variations in the concentrations of elements and the particular elements selected may be made. Of course, where such variations are made, it should be understood that such variations may have a desirable or undesirable effect on the steel sheet microstructure and/or mechanical properties in accordance with the properties described above for each given alloying addition.

### EXAMPLE 1

Examples of the steel sheet were made with the compositions set forth in Table 1 below.

The materials were processed on laboratory equipment according to the following parameters. Each sample was subjected to Gleeble 1500 treatments using copper cooled wedge grips and the pocket jaw fixture. Samples were austenitized at 1100 °C and then cooled to room temperature at various cooling rates between 1-100 °C/s.

**Table 1 Chemical compositions in weight %.**

| ID | Description | Al | C | Co | Cr | Cu | Mn | Mo | Nb | Ni | P | Si | Sn | Ti | V | W |
|---|---|---|---|---|---|---|---|---|---|---|---|---|---|---|---|---|
| V4037 | Lab Material | 1.41 | 0.19 | - | 0.01 | <0.003 | 1.54 | <0.003 | <0.003 | <0.003 | <0.003 | 0.11 | <0.003 | 0.01 | <0.003 | - |
| V4038 | Lab Material | 1.29 | 0.22 | - | 0.20 | <0.003 | 1.68 | <0.003 | 0.02 | <0.003 | 0.02 | 0.01 | <0.003 | 0.01 | <0.003 | - |
| V4039 | Lab Material | <0.003 | 0.20 | <0.002 | 0.01 | <0.002 | 2.94 | <0.002 | 0.00 | <0.002 | 0.00 | 1.57 | <0.002 | 0.01 | <0.002 | 0.00 |

### EXAMPLE 2

The Rockwell hardness of each of the steel compositions described in Example 1 and Table 1 above was taken on the surface of each sample. The results of the tests are plotted in FIGS. 3-5 with Rockwell hardness plotted as a function of cooling rate. The average of at least seven measurements is shown for each data point. The compositions V4037, V4038 and V4039 correspond to FIGS. 3, 4, and 5, respectively.

### EXAMPLE 3

Light optical micrographs were taken in the longitudinal through thickness direction near the center of each sample for each of the compositions of Example 1. The results of these tests are shown in FIGS. 6-8. The compositions V4037, V4038, and V4039 correspond to FIGS. 6, 7, and 8, respectively. Additionally, FIGS. 6-8 each contain six micrographs for each composition with each micrograph representing a sample subjected to a different cooling rate.

### EXAMPLE 4

A critical cooling rate for each of the compositions of Example 1 was estimated using the data of Examples 2 and 3 in accordance with the procedure described herein. The critical cooling rate herein refers to the cooling rate required to form martensite and avoid the formation of non-martensitic transformation products. The results of these tests are as follows:

| | |
|---|---|
| V4037: | 70 °C/s |
| V4038: | 75 °C/s |
| V4039: | 7 °C/s |

### EXAMPLE 5

Examples of the steel sheet were made with the compositions set forth in Table 2 below.

The materials were processed by melting, hot rolling, and cold rolling. The materials were then subjected to testing described in greater detail below in Examples 6-7. All of the compositions listed in Table 2 are comparative examples and were intended for use with the process described above with respect to FIG. 2 with the exception of V4039 which was intended for use with the process described above with respect to FIG. 1. Heat V4039 had a composition intended to provide higher hardenability as required by the thermal profile described above with respect to FIG. 1. As a result V4039 was subjected to annealing at 600 °C for 2 hours in 100% H2 atmosphere after hot rolling, but prior to cold rolling. All materials were reduced during cold rolling about 75% to 1mm. Results for some of the material compositions set forth in Table 2 after hot rolling and cold rolling are shown in Tables 3 and 4, respectively.

**Table 2 Chemical compositions in weight %.**

| **Heat** | **Description** | **C** | **Mn** | **Si** | **Al** | **Mo** | **Cr** | **Nb** | **B** |
|---|---|---|---|---|---|---|---|---|---|
| V4037 | Lab Material | 0.19 | 1.54 | 0.11 | 1.41 | 0 | 0.009 | 0 | 0.0007 |
| V1307 | Lab Material | 0.19 | 1.53 | 1.48 | 0.041 | 0 | 0 | 0 | 0.0005 |
| V4063 | Lab Material | 0.19 | 1.6 | 0.11 | 1.34 | 0 | 0.003 | 0 | 0.0007 |
| V4038 | Lab Material | 0.22 | 1.68 | 0.007 | 1.29 | 0 | 0.2 | 0.021 | 0.0008 |
| V4039 | Lab Material | 0.2 | 2.94 | 1.57 | <0.030 | <0.002 | 0.005 | 0.002 | N/R |
| A1305 | Lab Material | 0.2 | 2.94 | 1.57 | 0 | 0 | 0 | 0 | 0.0006 |
| V4107 | Lab Material | 0.18 | 4.03 | 1.63 | 0.005 | 0 | 0 | 0 | 0.0008 |
| V4108 | Lab Material | 0.18 | 5.06 | 1.56 | 0.004 | 0 | 0 | 0 | 0.0009 |
| V4060 | Lab Material | 0.4 | 1.2 | 1.97 | 0.003 | 0 | 0.19 | 0.007 | 0.0005 |
| V4061 | Lab Material | 0.41 | 1.2 | 0.98 | 0.003 | 0 | 0.003 | 0 | 0.0004 |
| V4062 | Lab Material | 0.39 | 1.18 | 0.012 | 1.16 | 0 | 0.003 | 0 | 0.0007 |
| V4078-1 | Lab Material | 0.2 | 1.67 | 0.1 | 1.41 | 0.28 | 0.003 | <0.003 | 0.0007 |
| V4078-2 | Lab Material | 0.2 | 1.67 | 0.1 | 1.41 | 0.27 | <0.003 | 0.051 | 0.0007 |
| V4079-1 | Lab Material | 0.19 | 1.94 | 0.098 | 1.43 | <0.003 | <0.003 | <0.003 | 0.0007 |
| V4079-2 | Lab Material | 0.19 | 1.96 | 0.099 | 1.41 | <0.003 | <0.003 | 0.051 | 0.0007 |

**Table 3 - Tensile Data, Post Hot Rolling**

| **Heat** | **YPE (%)** | **Upper YS** | | **Lower YS** | | **Yield Strength 0.2% Offset** | | **UTS** | | **Total Elongation (2")** | **Uniform Elongation %** | **Hardness HRA** |
|---|---|---|---|---|---|---|---|---|---|---|---|---|
| | | **MPa** | **ksi** | **MPa** | **ksi** | **MPa** | **ksi** | **MPa** | **ksi** | | | |
| V4063 | 0 | N/A | N/A | N/A | N/A | 375 | 54 | 652 | 95 | 26 | 15 | 53 |
| | 0 | N/A | N/A | N/A | N/A | 380 | 55 | 648 | 94 | 26 | 15 | 53 |
| V4039* | 0 | N/A | N/A | N/A | N/A | 640 | 93 | 1085 | 157 | 14 | 9 | 67 |
| V4039* (annealed) | 0 | N/A | N/A | N/A | N/A | 603 | 88 | 748 | 109 | 20 | 10 | 61 |
| V4060 | 0.6 | 645 | 94 | 637 | 92 | 633 | 92 | 883 | 128 | 20 | 11 | 63 |
| | 0.5 | 610 | 89 | 605 | 88 | 611 | 89 | 876 | 127 | 22 | 12 | 61 |
| V4061 | 0 | N/A | N/A | N/A | 0 | 496 | 72 | 790 | 115 | 22 | 11 | 60 |
| | 0 | N/A | N/A | N/A | 0 | 507 | 74 | 799 | 116 | 20 | 11 | 60 |
| V4062 | 1.1 | 507 | 74 | 501 | 73 | 506 | 73 | 712 | 103 | 26 | 12 | 60 |
| | 0.7 | 505 | 73 | 502 | 73 | 502 | 73 | 713 | 103 | 24 | 12 | 57 |
| V4078-1 | 0.8 | 427 | 62 | 416 | 60 | 425 | 62 | 594 | 86 | 32 | 18 | 51 |
| V4078-2 | 0.6 | 525 | 76 | 519 | 75 | 525 | 76 | 685 | 99 | 21 | 15 | 56 |
| V4079-1 | 1.8 | 364 | 53 | 361 | 52 | 361 | 52 | 544 | 79 | 30 | 17 | 48 |
| V4079-2 | 1.2 | 497 | 72 | 481 | 70 | 489 | 71 | 639 | 93 | 24 | 13 | 52 |

| | | | | | | | | | | | | |
|---|---|---|---|---|---|---|---|---|---|---|---|---|
| *Tensile test performed in transverse direction for V4039 | | | | | | | | | | | | |

**Table 4 - Tensile Data, Post Cold Rolling**

| **Heat** | **Yield Strength 0.2% Offset** | | **UTS** | | **Elongation (2") %** | **Uniform Elongation %** | **Hardness HRA** |
|---|---|---|---|---|---|---|---|
| | **MPa** | **ksi** | **MPa** | **ksi** | | | |
| V4037 | 927 | 134 | 971 | 141 | 4.8 | 1.4 | 64 |
| V4063 | 1046 | 152 | 1101 | 160 | 2.4 | 1.3 | 65 |
| V4038 | 1001 | 145 | 1054 | 153 | 5.5 | 1.6 | 65 |
| V4039 | 1149 | 167 | 1216 | 176 | 4.4 | 1.5 | 68 |
| V4060 | 1266 | 184 | 1393 | 202 | 5.4 | 1.9 | 69 |
| V4061 | 1187 | 172 | 1279 | 186 | 4.3 | 1.7 | 68 |
| V4062 | 1111 | 161 | 1185 | 172 | 4.3 | 1.7 | 66 |
| V4078-1 | 1047 | 152 | 1105 | 160 | 3.6 | 1.4 | 65 |
| V4078-2 | 1154 | 167 | 1209 | 175 | 4.2 | 1.4 | 66 |
| V4079-1 | 932 | 135 | 975 | 141 | 4.6 | 1.4 | 64 |
| V4079-2 | 1034 | 150 | 1078 | 156 | 3.9 | 1.3 | 66 |

### EXAMPLE 7

The compositions of Example 5 were subjected to Gleeble dilatomety. Gleeble dilatomety was performed in vacuum using a 101.6x25.4x1 mm samples with a c-strain gauge measuring dilation in the 25.4 mm direction. Plots were generated of the resulting dilation vs. temperature. Line segments were fit to the dilatometric data and the point at which the dilatometric data deviated from linear behavior was taken as the transformation temperature of interest (e.g., A₁, A₃, Mₛ). The resulting transformation temperatures are tabulated in Table 5.

Gleeble methods were also used to measure a critical cooling rate for each of the compositions of Example 5. The first method utilized Gleeble dilatomety, as described above. The second method utilized measurements of Rockwell hardness. In particular, after samples were subjected to Gleeble testing at range of cooling rates, Rockwell hardness measurements were taken. Thus, Rockwell hardness measurements were taken for each material composition with a measurement of hardness for a range of cooling rates. A comparison was then made between the Rockwell hardness measurements of a given composition at each cooling rate. Rockwell hardness deviations of 2 points HRA were considered significant. The critical cooling rate to avoid non-martensitic transformation product was taken as the highest cooling rate for which the hardness was lower than 2 point HRA than the maximum hardness. The resulting critical cooling rates are also tabulated in Table 5 for some of the compositions listed in Example 5.

**Table 5 - Transformation Temperatures and Critical Cooling Rate from Gleeble Dilatomety**

| **Heat** | **A₁ (°C)** | **A₃ (°C)** | **M, (°C)** | **Critical Cooling Rate (°C/s)** | |
|---|---|---|---|---|---|
| | | | | Gleeble Dilatometry | Gleeble/ Hardness |
| V4037 | 737 | 970 | 469 | Inconclusive | 65 |
| V4063 | 720 | 975 | 425 | 70 | - |
| V4038 | 791 | 980 | 441 | - | 65 |
| V4039 | 750 | 874 | 394 | <10 | 6 |
| V4060 | 725 | 975 | 325 | 30 | - |
| V4061 | 675 | 900 | 325 | 40 | 55 |
| V4062 | 700 | 975 | 375 | 30 | - |
| V4078-1 | 750 | 925 | 450 | 40 | 55 |
| V4078-2 | 790 | 980 | 425 | 40 | - |
| V4079-1 | 800 | 1000 | 430 | 40 | - |
| V4079-2 | 750 | 990 | 425 | 40 | - |

### EXAMPLE 8

The compositions of Example 5 were used to calculate quench temperature and a theoretical maximum of retained austenite. The calculations were performed using the methods of *Speer et al*., described above. The results of the calculations are tabulated below in Table 6 for some of the compositions listed in Example 5.

**Table 6 - Quench Temperature and Theoretical Maximum of Retained Austenite**

| **Heat** | **QT (°C)** | **f(y) Theoretical Maximum** |
|---|---|---|
| V4037 | 281 | 0.15 |
| V4063 | 278 | 0.15 |
| V4038 | 270 | 0.18 |
| V4039 | 203 | 0.2 |
| V4060 | 191 | 0.35 |
| V4061 | 196 | 0.36 |
| V4062 | 237 | 0.31 |
| V4078-1 | 276 | 0.16 |
| V4078-2 | 276 | 0.16 |
| V4079-1 | 273 | 0.16 |
| V4079-2 | 272 | 0.16 |

### EXAMPLE 9

The samples of the compositions of Example 5 were subjected to the thermal profiles shown in FIGS. 1 and 2 with peak metal temperature and quench temperature varied between samples of a given composition. As described above, only composition V4039 was subjected to the thermal profile shown in FIG. 1, while all other compositions were subjected to the thermal cycle shown in FIG. 2. For each sample, tensile strength measurements were taken. The resulting tensile measurements are plotted in FIGS. 9-12. In particular, FIGS. 9-10 show tensile strength data plotted against austenitization temperature and FIGS. 11-12 show tensile strength data plotted against quench temperature. Additionally, where the thermal cycles were performed using Gleeble methods, such data points are denoted with "Gleeble." Similarly, where thermal cycles were performed using a salt bath, such data points are denoted with "salt."

Additionally, similar tensile measurements for each composition listed in Example 5 (where available) are tabulated in Table 7, shown below. Partitioning times and temperatures are shown for example only, in other embodiments the mechanisms (such as carbon partitioning and/or phase transformations) occur during non-isothermal heating and cooling to or from the stated partitioning temperature which may also contribute to final material properties.

**Table 7 - Tensile Data, Post Partitioning**

| **Heat** | **Peak Metal Temp (°C)** | **Quench Temp (°C)** | **Partitioning Temp (°C)** | **Partitioning Time (s)** | **0.2% Yield Strength** | **Ultimate Tensile Strength** | **Total Elongation (%)** | **TE x UTS (Mpa x %)** |
|---|---|---|---|---|---|---|---|---|
| V1307 | 800 | 250 | 466 | 30 | 419 | 818 | 27 | 22,424 |
| | 800 | 250 | 466 | 30 | 416 | 807 | 28 | 22,345 |
| | 850 | 250 | 466 | 30 | 553 | 862 | 25 | 21,805 |
| | 850 | 250 | 466 | 30 | 535 | 847 | 25 | 21,336 |
| | 900 | 250 | 466 | 30 | 548 | 854 | 24 | 20,144 |
| | 800 | 250 | 400 | 30 | 445 | 898 | 22 | 19,675 |
| | 900 | 250 | 466 | 30 | 566 | 856 | 23 | 19,594 |
| | 800 | 250 | 400 | 30 | 432 | 889 | 22 | 19,478 |
| V4060 | 800 | 160 | 466 | 15 | 746 | 1317 | 23 | 29,630 |
| | 800 | 200 | 466 | 15 | 716 | 1332 | 19 | 25,309 |
| | 800 | 250 | 466 | 15 | 718 | 1403 | 18 | 25,115 |
| | 800 | 200 | 466 | 15 | 632 | 1309 | 19 | 24,746 |
| | 800 | 250 | 466 | 15 | 701 | 1379 | 18 | 24,407 |
| | 800 | 160 | 466 | 15 | 845 | 1311 | 18 | 23,986 |
| | 850 | 250 | 466 | 15 | 891 | 1291 | 18 | 23,749 |
| | 850 | 250 | 466 | 15 | 735 | 1223 | 19 | 23,729 |
| V4037 | 850 | 300 | 466 | 15 | 443 | 657 | 32 | 20,763 |
| | 921 | 200 | 466 | 30 | 325 | 612 | 34 | 20,633 |
| | 850 | 250 | 466 | 15 | 405 | 696 | 30 | 20,543 |
| | 921 | 300 | 466 | 30 | 380 | 591 | 34 | 20,090 |
| | 921 | 356 | 466 | 30 | 386 | 592 | 34 | 20,078 |
| | 921 | 400 | 466 | 30 | 388 | 588 | 34 | 19,937 |
| | 940 | 200 | 466 | 30 | 362 | 598 | 33 | 19,906 |
| | 850 | 200 | 466 | 15 | 427 | 687 | 28 | 19,022 |
| | 940 | 200 | 466 | 30 | 353 | 592 | 32 | 18,989 |
| | 980 | 200 | 466 | 30 | 341 | 612 | 31 | 18,897 |
| | 900 | 300 | 466 | 15 | 493 | 727 | 26 | 18,767 |
| | 850 | 200 | 466 | 15 | 447 | 702 | 27 | 18,600 |
| | 850 | 300 | 466 | 15 | 404 | 678 | 27 | 18,435 |
| | 980 | 200 | 466 | 30 | 347 | 611 | 30 | 18,387 |
| | 940 | 200 | 466 | 30 | 330 | 548 | 33 | 18,253 |
| | 980 | 200 | 466 | 30 | 345 | 612 | 29 | 17,939 |
| V4038 | 850 | 300 | 466 | 15 | 481 | 754 | 26 | 19,536 |
| | 918 | 400 | 466 | 30 | 377 | 681 | 27 | 18,461 |
| | 918 | 286 | 466 | 30 | 357 | 695 | 26 | 18,348 |
| | 918 | 200 | 466 | 30 | 363 | 697 | 26 | 18,193 |
| | 918 | 300 | 466 | 30 | 354 | 696 | 26 | 17,949 |
| | 850 | 300 | 466 | 15 | 457 | 773 | 23 | 17,777 |
| V4039 | 800 | 250 | 400 | 60 | 821 | 1299 | 15 | 19,225 |
| | 800 | 250 | 400 | 60 | 821 | 1298 | 15 | 18,945 |
| | 900 | 250 | 400 | 60 | 923 | 1273 | 15 | 18,593 |
| | 850 | 250 | 400 | 60 | 874 | 1278 | 14 | 18,142 |
| | 900 | 250 | 400 | 60 | 913 | 1258 | 14 | 17,984 |
| V4060 | 800 | 160 | 466 | 15 | 746 | 1317 | 23 | 29,630 |
| | 800 | 200 | 466 | 15 | 716 | 1332 | 19 | 25,309 |
| | 800 | 250 | 466 | 15 | 718 | 1403 | 18 | 25,115 |
| | 800 | 200 | 466 | 15 | 632 | 1309 | 19 | 24,746 |
| | 800 | 250 | 466 | 15 | 701 | 1379 | 18 | 24,407 |
| | 800 | 160 | 466 | 15 | 845 | 1311 | 18 | 23,986 |
| | 850 | 250 | 466 | 15 | 891 | 1291 | 18 | 23,749 |
| | 850 | 250 | 466 | 15 | 735 | 1223 | 19 | 23,729 |
| | 800 | 200 | 466 | 30 | 942 | 1319 | 17 | 22,422 |
| | 850 | 200 | 466 | 15 | 695 | 1222 | 16 | 19,070 |
| V4061 | 750 | 250 | 466 | 15 | 553 | 985 | 20 | 19,902 |
| | 750 | 250 | 466 | 15 | 581 | 918 | 21 | 18,996 |
| V4062 | 750 | 200 | 466 | 15 | 478 | 813 | 23 | 18,778 |
| | 750 | 250 | 466 | 15 | 480 | 816 | 22 | 17,944 |
| | 750 | 200 | 466 | 15 | 536 | 790 | 23 | 17,936 |
| V4107 | 850 | 250 | 400 | 60 | 776 | 1382 | 13 | 17,824 |
| V4108 | 900 | 250 | 400 | 60 | 923 | 1642 | 11 | 17,401 |
| | 850 | 250 | 400 | 60 | 952 | 1620 | 11 | 17,337 |
| V4078-1 | 850 | 300 | 466 | 15 | 448 | 783 | 24 | 19,016 |
| | 850 | 300 | 466 | 15 | 492 | 761 | 24 | 17,888 |
| V4078-2 | 900 | 250 | 466 | 30 | 713 | 843 | 21 | 17,946 |
| | 850 | 300 | 466 | 15 | 689 | 859 | 20 | 17,525 |
| | 850 | 300 | 466 | 15 | 671 | 871 | 20 | 17,503 |

The limits of this invention should be determined from the appended claims.

## Claims

1. A method for producing a hot dip galvanized/galvannealed steel sheet, the steel sheet consisting of the following elements by weight percent:
0.15-0.5% carbon;
1-3% manganese;
2% or less silicon, aluminum, or some combination thereof;
0.5% or less molybdenum;
0.05% or less niobium; and
the balance being iron and other incidental impurities;
or
0.15-0.4% carbon;
1.5-4% manganese;
2% or less silicon, aluminum, or some combination thereof;
0.5% or less molybdenum;
0.05% or less niobium; and
the balance being iron and other incidental impurities;
the method comprising the steps of:
(a) heating the steel sheet to a first temperature (T1), wherein T1 is at least above the temperature at which the steel sheet transforms to austenite and ferrite;
(b) cooling the steel sheet to a quench temperature by cooling at a cooling rate, wherein the quench temperature is below the martensite start temperature (Ms) as defined by Andrew's linear expression, wherein the difference between the quench temperature and Ms being sufficiently great to form an adequate amount of martensite yet being sufficiently low to avoid consuming too much austenite, wherein the cooling rate is sufficiently rapid to transform austenite to martensite, to avoid the formation of non-martensitic transformation products;
(c) re-heating the steel sheet to a partitioning temperature, wherein the partitioning temperature is sufficient to permit diffusion of carbon within the structure of the steel sheet;
(d) stabilizing austenite by holding the steel sheet at the partitioning temperature for a holding time, wherein the holding time is of a period of time sufficient to permit diffusion of carbon from martensite to austenite;
(e) subjecting the steel sheet to a hot dip galvanizing or galvannealing process during the step of stabilizing austenite; and
(f) cooling the steel sheet to room temperature.

2. The method of claim 1, wherein the hot dip galvanizing or galvannealing occurs above Ms.

3. The method of claim 1, wherein the partitioning temperature is above Mₛ.

## Patentansprüche

1. Ein Verfahren zur Herstellung eines feuerverzinktem/galvannealten Stahlblechs, wobei das Stahlblech aus den folgenden Elementen nach Gewichtsprozenten besteht: 0,15-0,5% Kohlenstoff;
1-3% Mangan;
2% oder weniger Silizium, Aluminium oder eine Kombination davon;
0,5% oder weniger Molybdän;
0,05% oder weniger Niobium; und
Rest Eisen oder andere übliche Verunreinigungen;
oder
0,15-0,4% Kohlenstoff;
1,5-4% Mangan;
2% oder weniger Silizium, Aluminium oder eine Kombination davon;
0,5% oder weniger Molybdän;
0,05% oder weniger Niobium; und
Rest Eisen oder andere übliche Verunreinigungen;
wobei das Verfahren die folgenden Schritte umfasst:
(a) Erhitzen des Stahlblechs auf eine erste Temperatur (T1), wobei T1 mindestens über der Temperatur ist, bei welcher das Stahlblech zu Austenit und Ferrit transformiert;
(b) Kühlen des Stahlblechs auf eine Quenchtemperatur durch Kühlen mit einer Kühlgeschwindigkeit, wobei die Quenchtemperatur unter der gemäß Andrew's linearer Expression definierten Martensit-Starttemperatur (Mₛ) liegt, wobei der Unterschied zwischen der Quenchtemperatur und Ms ausreichend groß ist ,um eine adäquate Menge Martensit zu bilden und doch niedrig genug ist, um den Verbrauch von zu viel Austenit zu vermeiden, wobei die Kühlgeschwindigkeit ausreichend schnell ist, um Austenit in Martensit zu transformieren, um die Bildung von nicht-martensitischen Transformationsprodukten zu vermeiden;
(c) Wiedererhitzen des Stahlblechs auf eine Partitionierungstemperatur, wobei die Partitionierungstemperatur ausreichend ist, um Diffusion von Kohlenstoff innerhalb der Struktur des Stahlblechs zu gestatten;
(d) Stabilisierung von Austenit mittels Haltens des Stahlblechs bei einer Partitionierungstemperatur für eine Haltezeit, wobei die Haltezeit eine Zeitspanne ist, welche ausreicht ist um Diffusion von Kohlenstoff von Martensit zu Austenit zu gestatten;
(e) Aussetzen des Stahlblechs einem Feuerverzinkungs- oder Galvannealingverfahrens währende des Schrittes der Austenitstabilisierung; und
(f) Abkühlen des Stahlblechs auf Raumtemperatur.

2. Das Verfahren nach Anspruch 1, wobei Feuerverzinkung oder Galvannealing oberhalb von Mₛ stattfindet.

3. Das Verfahren nach Anspruch 1, wobei, die Partitionierungstemperatur oberhalb von Mₛ ist.

## Revendications

1. Procédé pour produire une tôle d'acier galvanisée à chaud au trempé / recuite avec galvanisation, la tôle d'acier consistant en les éléments suivants, en pourcentages en poids :
0,15 à 0,5 % de carbone ;
1 à 3 % de manganèse ;
2 % ou moins de silicium, d'aluminium, ou d'une combinaison de ceux-ci ;
0,5 % ou moins de molybdène ;
0,05 % ou moins de niobium ; et
le reste étant du fer et d'autres impuretés accidentelles ;
ou
0,15 à 0,4 % de carbone ;
1,5 à 4 % de manganèse ;
2 % ou moins de silicium, d'aluminium, ou d'une combinaison de ceux-ci ;
0,5 % ou moins de molybdène ;
0,05 % ou moins de niobium ; et
le reste étant du fer et d'autres impuretés accidentelles ;
le procédé comprenant les étapes suivantes :
(a) chauffage de la tôle d'acier à une première température (T1), laquelle T1 est au moins supérieure à la température à laquelle la tôle d'acier se transforme en austénite et ferrite ;
(b) refroidissement de la tôle d'acier à une température de trempe par refroidissement à une certaine vitesse de refroidissement, laquelle température de trempe est inférieure à la température de début de martensite (Mₛ) telle que définie par l'expression linéaire d'Andrew, la différence entre la température de trempe et Mₛ étant suffisamment importante pour qu'il se forme une quantité de martensite adéquate tout en étant suffisamment faible pour éviter que trop d'austénite soit consommée, laquelle vitesse de refroidissement étant suffisamment élevée pour que l'austénite se transforme en martensite, afin que soit évitée la formation de produits de transformation non martensitiques ;
(c) nouveau chauffage de la tôle d'acier à une température de séparation, laquelle température de séparation est suffisante pour que soit permise la diffusion de carbone dans la structure de la tôle d'acier ;
(d) stabilisation de l'austénite par maintien de la tôle d'acier à la température de séparation pendant un certain temps de maintien, lequel temps de maintien est une période de temps suffisante pour que soit permise la diffusion de carbone de la martensite à l'austénite ;
(e) soumission de la tôle d'acier à un traitement de galvanisation à chaud au trempé ou de recuit avec galvanisation durant l'étape de stabilisation de l'austénite ; et
(f) refroidissement de la tôle d'acier à la température ambiante.

2. Procédé selon la revendication 1, dans lequel la galvanisation à chaud au trempé ou le recuit avec galvanisation a lieu au-delà de Mₛ.

3. Procédé selon la revendication 1, dans lequel la température de séparation est supérieure à Mₛ.
